

## UNITED STATES PATENT OFFICE.

LEWIS C. MAY, OF COCHITUATE, MASSACHUSETTS.

## IMPROVEMENT IN COMPOSITIONS FOR COLORING LEATHER.

Specification forming part of Letters Patent No. 124,965, dated March 26, 1872.

Specification describing a new and useful Improvement in Composition for Leather, invented by LEWIS C. MAY, of Cochituate, in the county of Middlesex and State of Massachusetts.

This invention relates to a compound to be applied to leather in the manufacture of boots and shoes, and for leather used for other purposes, for changing the color or complexion of the leather, designed more especially for changing the color of the soles or bottoms of boots and shoes, but not confined thereto; and it consists in a compound composed of the ingredients hereinafter named, combined in about the proportions and in about the manner specified.

In carrying out my invention and discovery, I take two gallons rye-flour paste; two gallons tragacanth paste; one pound American isinglass; one and one-fourth pound oxalic acid; one-fourth pound gum gamboge; three pounds pipe-clay, united with water sufficient to make ten gallons of the compound of the proper consistency for use.

The mode of preparation is substantially as follows: While the rye paste (made in the usual way) is hot, add the isinglass and stir until all is dissolved; then add the tragacanth paste; then let the mass cool, and, when cold, add the

oxalic acid, gum gamboge, and pipe-clay and water. Let the composition stand for the space of a week or so before using.

This composition fills the pores and makes the leather bright and hard. By the use of a revolving brush, or friction applied otherwise after the application of the composition, the complexion or color of the leather may be changed, as desired. The bottom of a boot or shoe or other leather may be made of a very light color, or of a dark red or other complexion or shade. This color, whichever it may be, will not fade, but improves the wear or durability of the leather.

I do not confine myself to the exact proportions named of the different ingredients, as they may be varied without departing from my invention.

Having thus described my invention, I claim as new and desire to secure by Letters Patent—

The composition above described, substantially as and for the purposes herein set forth.

LEWIS C. MAY.

Witnesses:

ADONIRAM J. PUFFER,  
JOHN C. BUTTERFIELD.